

## 1

3,216,937

**LUBRICANT FOR MARINE DIESEL ENGINES**  
Arnold J. Morway, Clark, and Fredrick L. Jonach, Short  
Hills, N.J., assignors to Esso Research and Engineering  
Company, a corporation of Delaware  
No Drawing. Filed Dec. 7, 1962, Ser. No. 242,930  
2 Claims. (Cl. 252—39)

This invention relates to lubricants. Particularly, the invention relates to lubricating oil compositions, having good antiwear properties, comprising mineral oil and alkaline earth metal salts of acetic acid and dicarboxylic acid.

While generally useful as lubricants for a variety of purposes, lubricants can be made according to the invention which are particularly effective for cylinder lubrication of marine diesel engines. Although marine diesel engines have become wide spread in their use, in these engines there has always been a serious wear problem with regard to the piston, the piston rings and the surface of the cylinder liner.

In lubricating these diesel engines, a fluid or semi-fluid lubricant is sprayed or forced directly onto the cylinder upon each stroke of the piston by means of a centralized forcefeed lubrication system. The lubricant is to a large extent consumed during each stroke of the piston, thereby requiring continuous application of the lubricant.

In order to be suitable for such lubrication use, the lubricant should have a fluid or semi-fluid consistency. This is desired in order that the lubricant may be readily pumped through the aforementioned forced lubrication systems normally associated with marine diesel engines and will spread or wet the piston sufficiently during each stroke to achieve an overall coating on the piston surface. As indicated above, another requirement of such lubricants is that they have good antiwear properties. Because of the giant size of the pistons and cylinders used in such engines (e.g. piston and cylinder diameters of about 36 inches are common), wear is a serious problem. Once the cylinder liner has worn more than about 0.6% of its diameter, it is necessary that it be replaced. In a typical marine engine of 8 to 16 cylinders such replacement cost may run in the order of several thousand dollars per cylinder. Wear of the piston and rings is also an expensive problem. The lubricant should also be storage stable, even when subject to long periods of vibration as occurs during storage in a ship's engine room.

Lubricants for such marine diesel lubrication, which met the above requirements, have been made by thickening mineral lubricating oil with mixed calcium salts of acetic acid and an intermediate molecular weight fatty acid, e.g.  $C_7$  to  $C_{10}$  or  $C_{12}$  fatty acids. It has now been found that marine diesel lubricants superior in several respects to those made from the intermediate molecular weight fatty acids and acetic acid, can be prepared by using dicarboxylic acid in place of part or all of the intermediate molecular weight fatty acid. By the use of the dicarboxylic acid, marine diesel lubricants can be prepared which are superior to said intermediate fatty acid type lubricant by having a reduced tendency to gel under hot conditions. Thus, in some engines operating at very high temperatures, gelling of the lubricant will interfere with the spreading of the lubricant onto the piston and cylinder, and will also interfere with pumping the lubricant through narrow diameter feed lines. In addition, in general the use of dicarboxylic acid results in a better

## 2

dispersion of calcium acetate, greater fluidity, and improved spreadability than is obtained by use of said aforementioned monocarboxylic acids.

The dicarboxylic acids operable in the invention include 5 those of the formula:



wherein R is a  $C_8$  to  $C_{20}$  aliphatic hydrocarbon group, either branched or straight chain, saturated or ethylenically unsaturated. Preferably R is a  $C_8$  to  $C_{12}$  saturated straight chain hydrocarbon group. Examples of such dicarboxylic acids include: sebacic acid, dodecanedioic acid,  $C_{19}$  dicarboxylic acid formed by the Koch process (this latter acid is slightly branched), etc.

10 The alkaline earth metal component of the mixed salt composition is preferably calcium since it results in the production of stable lubricants having load carrying and antiwear characteristics even without the use of conventional extreme pressure and stabilizing agents. The other 15 alkaline earth metals such as barium, strontium and magnesium can be used, but are not as good as calcium in these respects.

15 The mixture of alkaline earth metal salts of the invention can be prepared by neutralization of acetic acid or 20 acetic anhydride and dicarboxylic acid with suitable bases, particularly hydrated lime. The neutralization step can be carried out in situ in the oil menstruum to which the 25 mixture of salts is to be applied in actual use, usually followed by dehydration by heating to about  $250^\circ$  to 30 about  $350^\circ$  F. until the salt mixture is substantially anhydrous, i.e. there is no free or unbound water present. It 35 is generally desirable to use a slight excess of base, e.g. lime, in order to form a slightly alkaline final product, e.g. 0.05 to 0.2 wt. percent alkalinity as measured in terms of NaOH. This alkalinity helps to neutralize corrosive acids formed by degradation of the lubricant during use and also imparts greater stability of the lubricant. Also 40 the alkalinity helps to neutralize corrosive sulfur-containing acids that may form upon combustion of high sulfur content fuel oil.

45 The mixture of alkaline earth metal salts of the invention can also be prepared by first forming at least a portion of the salt of the dicarboxylic acid in oil, then forming the acetate salt by neutralization in the presence of 50 dicarboxylic acid salt, then heating under substantially dehydration conditions. This method is believed to result in a more stable lubricant since dicarboxylic acid salt is believed to limit the crystal growth of the acetate salt particles which are subsequently formed by the neutralization 55 of the acetic acid with metal base. Also, when using lime, it is generally desirable to carry out the bulk of the neutralization with insufficient lime present so that the excess acid will react with any carbonates that may be present in commercial lime, then adding a small amount of additional lime to completely neutralize the acids and preferably to also form an alkaline product.

60 The mixed salt lubricants of the invention can be prepared by using 1 to 100, preferably 5 to 40, molar hydrogen equivalents of acetic acid or acetic anhydride per molar hydrogen equivalent of dicarboxylic acid. For lubricants designed for marine diesel lubrication, good results are obtained by using a ratio of about 5 to 15 molar hydrogen equivalents of the acetic acid or its anhydride per molar hydrogen equivalent of dicarboxylic acid.

65 The finished lubricant will generally be a fluid or semi-fluid comprising a major amount of lubricating oil and about 3 to 20, preferably 5 to 12 wt. percent of the mixed

salt combination. For economy purposes in heating during large scale manufacture, concentrates of 20 to 45 wt. percent of the mixed salts in oil can be made by the in situ technique, after which the concentrate is diluted with additional oil to form the finished lubricant. This dilution is readily made by adding the additional oil and mixing. Both the concentrate and finished lubricant can be homogenized in a Morehouse mill, Charlotte mill, Gaulin homogenizer, etc. If enough of the mixed salt is used in the oil, a soft solid grease is obtained. However, these greases do not seem to have very good structural stability. As a result, the mixed salt composition of the invention is preferably used in the form of fluid or semi-fluid lubricant.

Mineral oil is the preferred lubricating oil, although various synthetic oils such as polysilicone, silanes, esters, Ucons, etc. may be used for special uses.

Various additives can be added to the finished lubricant in amounts of 0.1 to 10.0 wt. percent, based on the weight of the finished lubricant. Among additives that can be added are corrosion inhibitors such as sodium nitrite, lanolin, wool grease stearin; antioxidants such as phenyl-alpha-naphthylamine; extreme pressure agents; dyes; etc.

The invention will be further understood by references to the following examples which include preferred embodiments of the invention.

#### EXAMPLE I

(All parts by weight)

9.45 parts of hydrated lime and 69.3 parts of a mineral lubricating oil having a viscosity of 80 SUS at 210° F. were added to a steam jacketed grease kettle and intimately mixed to a smooth slurry. Then 1.14 parts of 1,12-dodecanedioic acid was added, with mixing. Mixing was continued for 1/2 hour, following which 16 parts of glacial acetic acid was slowly added while mixing over a period of another 1/2 hour. All of this mixing was carried out by circulating the grease from the grease kettle through a Charlotte mill having an 0.005" clearance. After the composition has been thus thoroughly mixed, 2.66 parts of dodecanedioic acid were added and the temperature of the mixture was raised by heating to 205° F. Then 1.05 parts of additional lime was added to give a free alkalinity content of 0.1 wt. percent determined as NaOH. All during the preceding period, the grease was continuously circulated through said Charlotte mill. The temperature of the grease was next raised to about 310° F. without milling. The temperature at 310° F. was held for 30 minutes, after which the grease was cooled by passing water through the kettle jacket. Upon cooling the grease to 200° F., 0.4 part of phenyl-alpha-naphthylamine was added as an oxidation inhibitor. The grease was further cooled to 100° F. where it was again milled by passage through the Charlotte mill. The resulting product was an excellent smooth grease having a consistency of a very viscous fluid. 1 part of this grease was then mixed with 3 parts of additional mineral lubricating oil of 80 SUS viscosity at 210° F. The diluted product was then passed through a Charlotte mill having a clearance of 0.003" after which the product was filtered through a 60 mesh screen and then packaged.

#### COMPARISON LUBRICANT

For comparison, a marine diesel cylinder lubricant was prepared by coneutralizing acetic acid and Wecoline AAC acid with lime in a mineral lubricating oil. A mole ratio of 12 molar hydrogen equivalent proportions of acetic acid per molar hydrogen equivalent of Wecoline AAC acid had been found to give the best overall results in a marine diesel cylinder lubricant. Wecoline AAC acid is a commercial acid derived from coconut oil and consisting of about 46 wt. percent capric acid, about 28 wt. percent caprylic acid and about 26 wt. percent lauric

acid. The comparison composition was dehydrated at a temperature of about 320° F. The product was homogenized by passage through a Morehouse mill.

The products prepared above and their properties are summarized in the following table:

| Finished Formulates (wt. percent)                                  | Example I                     | Comparison           |
|--------------------------------------------------------------------|-------------------------------|----------------------|
| Acetic Acid (glacial).....                                         | 4.00.....                     | 3.84.                |
| Dodecanedioic Acid.....                                            | .95.....                      | 0.93.                |
| Wecoline AAC Acid.....                                             | 2.55.....                     | 2.70.                |
| Hydrated Lime.....                                                 | 0.10.....                     |                      |
| Phenyl $\alpha$ -naphthylamine.....                                | 92.40.....                    | 92.53.               |
| Mineral Lubricating Oil, 55 SUS at 210° F.....                     | 8/1.....                      | 12/1.                |
| Molar hydrogen equivalent ratio, acetic/higher acids.              |                               |                      |
| Properties:                                                        |                               |                      |
| Appearance.....                                                    | Uniform, fluid slight opaque. | Uniform, semi-fluid. |
| Vis./100° F. SUS.....                                              | 1,029.....                    | 1,787.               |
| Vis./210° F. SUS.....                                              | 78.1.....                     | 138.8.               |
| Base No. ASTM D664 mm.                                             | 42.5.....                     | 29.6.                |
| KOH/gm.                                                            | 0.65.....                     | 0.8.                 |
| Centrifuge Test, Percent Sediment, 1,500 r.p.m.—4 hours.           |                               |                      |
| Oven Test, 4 hours at 350° F.                                      |                               |                      |
| 4-Ball Wear Test, scar diam., mm., 1 hr.—1,800 r.p.m.—10 kg. Load. |                               |                      |
| 100 Mesh Screen Test.....                                          | Readily passes through.       | Passes through.      |
| Manzell Lubrication Test.....                                      | 120 days.                     | 18 days.             |
| Thermal Stability Test:                                            |                               |                      |
| @ 150° C.....                                                      | Fluid.....                    | No gel.              |
| @ 190° C.....                                                      | Fluid.....                    | Gel.                 |

The products of Example I gave a very low wear scar diameter of 0.23 mm. in the 4-Ball Wear Test as compared to a scar diameter of 0.30 mm. for the comparison lubricant.

The Manzell Lubricator test of Table I is carried out by passing the lubricant under test through a Manzell Lubricator at the rate of 2 quarts of lubricant a day. The Manzell Lubricator includes a sight-glass filled with an aqueous solution containing 50 wt. percent of a calcium nitrate tetrahydrate as the sight-glass fluid. These lubricators are widely used in conjunction with marine diesel engines. The lubricator permits visual observation of the rate of flow of the lubricant which is forced into the bottom of the sight-glass and then floats up through the higher density sight-glass fluid to an upper line from where it is then forced to the cylinder being lubricated. The product of Example I went for 120 days without fogging the sight-glass. On the other hand, the comparison lubricant went for only 18 days before the sight-glass had become sufficiently fogged so as to require disassembling and cleaning.

The Thermal Stability test was carried out by filling an ASTM pour point jar 3/4 full with the lubricant to be tested. The test lubricant was heated for four hours and is then cooled for 45 minutes. The jar is then examined to see if the lubricant has gelled. It is seen that at the 190° C. heating level, that the comparison lubricant had gelled while the product of Example I had not. This gelling or lack of gelling is used as an indication of the spreading ability of the lubricant when it hits the hot cylinder it is being used to lubricate. For example, a cylinder at a temperature of 190° C., when hit by the comparison lubricant of Table I would cause the lubricant to gel so as to interfere with the spreadability of the lubricant along the cylinder walls. On the other hand, the product of Example I will not form a gel at this temperature and as a result will remain fluid so that it can rapidly spread along the cylinder to more evenly wet the cylinder with the lubricant.

The Hot Plate Spread Test is carried out by simply allowing drops of the lubricant to fall on a hot iron surface at 450° F. and observing whether or not the lubricant spreads or gels.

The data of the table shows that the product of the invention resulted in a lubricant which was more fluid,

more stable against sedimentation as measured by the Centrifuge Test, did not gel on a hot iron surface at 450° F. or in the Thermal Stability Test, gave lower wear and was slower to foul the Manzell Lubricator than the comparison lubricant.

The table also demonstrates the lower thickening power of the dicarboxylic acid salt as compared to the monocarboxylic acid Wecoline salt. This represents a major advantage for many types of uses, since it permits the incorporation of large amounts of calcium acetate salt into oil with relatively little thickening. Thus, the excellent anti-wear properties imparted by calcium acetate can be incorporated into oil to form more fluid lubricants than could generally be heretofore obtained.

What is claimed is:

1. A fluid marine diesel cylinder lubricant having a reduced tendency to gel at high temperatures consisting essentially of a major proportion of mineral lubricating oil and about 5 to 12 wt. percent of calcium salt of acetic acid and  $C_{10}$  to  $C_{14}$  unsubstituted saturated aliphatic dicarboxylic acid in a molar hydrogen equivalent ratio of

10

15

20

said acetic acid to said dicarboxylic acid of about 5:1 to 15:1.

2. A fluid marine diesel cylinder lubricant having a reduced tendency to gel at elevated temperatures consisting essentially of a major proportion of mineral lubricating oil and about 5 to 12 wt. percent of calcium salt of acetic acid and dodecanedioic acid in a molar hydrogen equivalent ratio of said acetic acid to said dicarboxylic acid of about 5:1 to 15:1.

References Cited by the Examiner

UNITED STATES PATENTS

|           |       |                         |            |
|-----------|-------|-------------------------|------------|
| 2,363,514 | 11/44 | Farrington et al. ----- | 252—40.7   |
| 2,699,428 | 1/55  | Lux et al. -----        | 252—39     |
| 2,846,392 | 8/58  | Morway et al. -----     | 252—39 X   |
| 2,859,179 | 11/58 | Lux et al. -----        | 252—39 X   |
| 2,976,242 | 3/61  | Morway -----            | 252—39 X   |
| 3,002,926 | 10/61 | Bergen -----            | 252—40.7 X |
| 3,071,547 | 1/63  | Morway -----            | 252—39     |

DANIEL E. WYMAN, Primary Examiner.